

# UNITED STATES PATENT OFFICE.

JOHN W. FRIES, OF WINSTON SALEM, NORTH CAROLINA.

## INDIGO DYE.

No. 807,453.

Specification of Letters Patent.

Patented Dec. 19, 1905.

Application filed October 12, 1904. Serial No. 228,196.

*To all whom it may concern:*

Be it known that I, JOHN W. FRIES, of Winston Salem, county of Forsyth, State of North Carolina, have invented an Improvement in 5 Indigo Dyes, of which the following is a specification.

My invention has reference to indigo dyes, and consists of certain improvements, which are fully set forth in the following specification.

In another application, Serial No. 227,098, and filed October 4, 1904, I have described a method of dyeing textile material with reduced indigo dyes and in connection therewith have specified the mixture of indigo dye forming the subject-matter of this application.

Heretofore the results with indigo in the art of dyeing have been, if applied to cotton yarn or fabrics in a strong or concentrated 20 "reduced" solution and then "oxidized" by exposure to the air or otherwise, the indigo is oxidized on the fiber superficially, and hence crocks badly and scours badly. If the dyeing is done by repeated dips in a dilute reduced 25 solution or a succession of comparatively dilute solutions, the result is much better as to fastness to rubbing and scouring; but it is impossible to exhaust an ordinary indigo-vat entirely, and if the weak indigo solution be 30 run off there is considerable waste. Further, very serious practical difficulties are experienced in the effort to "feed" indigo, so as to keep up a standing vat. This is due to the fact that the reduced solution of indigo and 35 the chemicals used for reduction are so unstable and are spontaneously decomposed, and, further, because the bath becomes saturated by these chemicals—*e. g.*, with the salts of iron or lime, zinc, and soda.

I have found it advantageous to apply to the dry yarn or fabric a reduced solution of indigo of such strength as is proportionate to the shade required by giving only one or two dips in this solution and expressing the surface 45 plus dye by squeeze-rollers, an operation familiarly known as "padding." For a full shade I prefer to use a padding liquor containing, for example, twenty pounds of indigo paste of twenty per cent. strength, or 50 four pounds of indigo-powder; twelve pounds of unslaked lime, which is to be slaked in sufficient water and the "milk of lime" used; four pounds zinc-dust; two pounds caustic soda, solid or granulated; two pounds starch, 55 and two pounds alizarin-oil, seventy-five per cent., the whole made up to twelve and one-

half gallons with water of preferably 120° to 140° Fahrenheit. In the preferred form of my composition I employ a mixture of the dry indigo-powder, zinc-dust, caustic soda, 60 sifted lime, and starch, substantially in the proportions specified, which may be sold as a commercial compound and mixed with water for use. A solution thus compounded will be found to "go on" or penetrate the fiber well; 65 but if exposed to the air, or if immersed in clear water, or in many solutions the indigo is oxidized on the fiber superficially. I convey the padded yarn directly from the squeeze-rolls of this padding liquor into a compartment containing a solution which will prevent this oxidation, and there the indigo is fixed upon or 70 "worked into" the fiber, and the result is a color much brighter and faster than can be obtained without this treatment. A dilute solution of hydrosulfite of soda is efficient for this 75 operation, or a solution of sodium sulfid may be used, which is still cheaper and easier of application. Other solutions having a reducing action or which will prevent the oxidation of the indigo during this operation may be substituted. After giving the yarn or 80 fabric the desired number of dips in this solution and passing through the proper squeeze-rolls the material is passed over reels 85 in the air to oxidize the indigo. It may then be rinsed or soaped, if desired, and dried. All these operations are preferably done in one continuous succession on machines of 90 simple construction.

While there are well-known ways of reducing indigo other than with zinc-dust and lime, I consider this the best because of cheapness, quickness, and ease of manipulation. Moreover, it appears to be the only manner of reducing indigo which admits of the ingredients being mixed together dry, if the alizarin-oil be left out; but in this case about four pounds of dry indigo-powder should be used instead of the twenty pounds of paste, as 95 stated in the formula.

Synthetic indigo is made in a dry powder; but it is almost universally used in the paste form, and it is recommended in this form by the manufacturers, because, as they say, the 105 powder needs to be ground into a paste with water before it can be properly used in making up an indigo-vat. The practical reason for this is that the dry powder is somewhat hard to mix with water in such fine subdivision and suspension in the water as to get thorough reduction; but I have found ex- 110

perimentally that if it be intimately mixed with the other ingredients, especially the starch, there is no difficulty in holding them all in suspension in the water with complete and rapid reduction of the indigo. As far as I am aware this use of starch is new and original, and I have introduced it for the double purpose of giving "body" to the solution to hold the other bodies in suspension until the indigo is reduced and also because the starch aids the penetration of the dye materially. The starch is insoluble in cold water ordinarily but it is soluble in cold caustic-alkali solutions, and we here have the caustic alkali, primarily, for the good it does the indigo solution, and, secondarily, as a solvent for the starch.

While I have given the proportions which I have found most advantageous, I do not restrict myself to these proportions as variations of them may reasonably be made. It

is also to be understood that my invention includes the use of the indigo either as a powder or as a paste, as may be desired.

Having now described my invention, what I claim as new, and desire to secure by Letters Patent, is—

1. A padding liquor for indigo - dyeing which consists of a mixture of indigo, milk of lime, zinc-dust, caustic soda, and starch, when mixed with a solvent.

2. A padding liquor for indigo - dyeing which consists of a mixture of indigo, milk of lime, zinc-dust, caustic soda, starch, and alizarin - oil, when mixed with water to form a solution.

In testimony of which invention I have hereunto set my hand.

JOHN W. FRIES.

Witnesses:

CHAS. A. WATSON,  
BERNARD J. PFOLEL.